

Patented Nov. 22, 1927.

## UNITED STATES PATENT OFFICE.

HUBERT H. CHAMPNEY, OF KENVIL, NEW JERSEY, ASSIGNOR TO HERCULES POWDER COMPANY, OF WILMINGTON, DELAWARE, A CORPORATION OF DELAWARE.

## EXPLOSIVE.

No Drawing.

Application filed May 8, 1925. Serial No. 28,958.

My invention relates to an improvement in explosives and more particularly to an improvement in permissible explosives.

The so-called permissible explosives when subjected to relatively high atmospheric temperatures, such as, for example, are encountered during the summer season, become hard or insensitive to detonation with a blasting cap. As a result of this tendency of the so-called permissible explosives, they are, during the summer season, unreliable.

Now it is the object of my invention to provide an explosive which will fall in the so-called permissible class, but which will not become hard or insensitive when subjected to relatively high atmospheric temperatures.

The ordinary so-called permissible explosive is composed, for example, of nitroglycerine, nitrate of ammonia, sodium nitrate and a carbonaceous ingredient as sawdust, pulp or ivory button meal. For the nitroglycerine may be substituted, in whole or in part, nitropolyglycerins, nitroglycols, or mixtures, or nitrosugars or nitroaromatic compounds, or mixtures in solution in nitroglycerine.

In accordance with my invention, I utilize ground oat hulls as an ingredient in the so-called permissible explosive in substitution, in whole or in part, for the carbonaceous ingredients, as sawdust, pulp, or ivory nut meal.

Ground oat hulls, as is well known, comprise the hulls of oats and I have found that they may be utilized in varying proportions of (say) from two per cent to eighteen per cent by weight, depending upon whether they displace all or only a part of the carbonaceous ingredients, and will prevent setting or loss of sensitiveness toward a blasting cap, when the explosive is subjected to elevated temperatures.

Explosives in accordance with my invention may, for example, comprise, in addition to ground oat hulls from 2%-18%, a sensitizer as nitroglycerine, by which I mean to include nitroglycerine, nitropolyglycerines, nitroglycols, or mixtures, nitrosugars, or nitroaromatic compounds in solu-

tion in nitroglycerine, or mixtures, say about 10%; an explosive, as ammonium nitrate, say 50%-80%; sodium nitrate, say up to 22%; carbonaceous ingredients as wood pulp, say 6% or less; and ivory nut meal, say 2% or less. The following formulæ may be stated by way of example:

|                  | Per cent. | Per cent. |
|------------------|-----------|-----------|
| Nitroglycerine   | 10        | 10        |
| Ammonium nitrate | 80        | 50 60     |
| Sodium nitrate   |           | 22        |
| Wood pulp        | 6         |           |
| Ivory meal       | 2         |           |
| Ground oat hulls | 2         | 18        |
|                  | —         | 65        |
|                  | 100       | 100       |

It will be understood that I do not intend that my invention shall be limited to the use of any particular proportions of ground oat hulls, nor to explosives having ingredients in the exact proportions above stated by way of example.

Having now fully described my invention, what I claim and desire to protect by Letters Patent is:

1. In an explosive in admixture, an explosive ingredient, a sensitizer, and ground oat hulls.
2. In an explosive in admixture, nitroglycerine about 10%, ammonium nitrate, and ground oat hulls from 2%-18%.
3. In an explosive in admixture, nitroglycerine about 10%, ammonium nitrate from 50%-80%, and ground oat hulls from 2%-18%.
4. In an explosive in admixture, nitroglycerine about 10%, ammonium nitrate about 50%, sodium nitrate about 22%, and ground oat hulls about 18%.
5. In an explosive in admixture, ammonium nitrate, a sensitizer and ground oat hulls.
6. In an explosive in admixture, ammonium nitrate, sodium nitrate, a sensitizer and ground oat hulls.
7. In an explosive in admixture, ammonium nitrate, a sensitizer and ground oat hulls from 2%-18%.

8. In an explosive in admixture, ammonium nitrate, sodium nitrate, a sensitizer and ground oat hulls from 2%-18%.
9. In an explosive in admixture, nitro-glycerine about 10%, ammonium nitrate from 50%-80%, ground oat hulls not less than 2% and other carbonaceous material not over 8%.
10. In an explosive in admixture, ammonium nitrate, a sensitizer, ground oat hulls and other carbonaceous material.

In testimony of which invention, I have hereunto set my hand, at Kenvil, New Jersey on this 2nd day of May, 1925.

HUBERT H. CHAMPNEY.